

1

3,411,914

**METHOD FOR STABILIZING X-RAY EMULSIONS  
TO RED SAFELIGHTS**

Claude Dostes, Joinville-le-Pont, France, assignor to Eastman Kodak Company, Rochester, N.Y., a corporation of New Jersey  
No Drawing. Filed July 13, 1964, Ser. No. 382,407  
Claims priority, application France, Dec. 5, 1963,  
956,168  
6 Claims. (Cl. 96—101)

**ABSTRACT OF THE DISCLOSURE**

Photographic silver halide emulsions are prepared by adding, after the end of the after-ripening step, first a tetraazaindene salt and then a noble metal salt. These emulsions have good sensitivity to image-forming radiation such as X-ray intensifier screen emissions and are substantially insensitive to red safelights.

This invention relates to photographic emulsions, and more particularly to photographic emulsions containing tetraazaindene antifoggants, which emulsions are not fogged by red safelights.

It is known to incorporate various tetraazaindene compounds, such as tetraazaindene salts, in photographic emulsions as antifoggants. While these compounds provide good fog control, they absorb some red radiation causing fog in the emulsion when handled in the presence of conventional red safelights. It therefore appears desirable to provide emulsions containing tetraazaindene salt antifoggants, which emulsions are not fogged by red radiation such as that emitted from red safelights.

One object of my invention is to provide photographic emulsions containing tetraazaindene salts, which emulsions are substantially insensitive to commonly employed red safelights. Another object of my invention is to provide a method of preparing photographic emulsions containing tetraazaindene salts, which emulsions are substantially insensitive to red radiation such as that emitted by commonly employed photographic red safelights. Other objects of my invention will appear herein.

These and other objects of my invention are accomplished by providing photographic emulsions which contain a noble metal salt and a tetraazaindene salt which is an antifoggant for photographic silver halide emulsions.

The preparation of silver halide emulsions involves three separate operations: (1) the emulsification and digestion or ripening of the silver halide; (2) the freeing of the emulsion from aqueous soluble salts usually by washing; and (3) the second digestion or after-ripening to obtain increased sensitivity (Mees, *The Theory of the Photographic Process*, 1954, p. 4). In accordance with my invention, the noble metal salt and tetraazaindene salt are incorporated in the emulsion subsequent to the after-ripening step or second digestion. In order to obtain satisfactory results, it is necessary to first add the tetraazaindene salt to the emulsion, and then the noble metal salt, followed by a short period of digestion.

The addition of only a gold salt (or noble metal) salt to an emulsion at the end of the after-ripening step, or thereafter, lowers the sensitivity of the emulsion to red radiation, but causes an undesirable desensitization of the emulsion to image-forming radiation. However, the addition of tetraazaindene salt and noble metal salt in that order subsequent to after-ripening of an emulsion provides an emulsion having good sensitivity to image-forming radiation and which is substantially insensitive to red radiation.

My invention will be further illustrated by the following example.

2

**EXAMPLE I**

A coarse grain silver bromoiodide emulsion of the type used in medical X-ray films was prepared in the customary manner, sulfur sensitized in accordance with Sheppard U.S. Patent 2,410,689, and after the second digestion, while the emulsion was cooling at a temperature of about 50° C., 1 gram 4-hydroxy-6-methyl-1,3,3a,7-tetraazaindene sodium salt per mole silver was incorporated in the emulsion, and immediately thereafter 1.3 mg. potassium chloroaurate per mole of silver was added to the emulsion. The temperature of the emulsion was held at about 50° C. for about 10 minutes, and then allowed to cool. The emulsion was coated on a support and subjected to radiation from a commonly used red safelight. The emulsion was found to be essentially free from fog whereas a control emulsion, which was the same as the test emulsion except that the noble metal salt was added before the tetraazaindene salt, was badly fogged when tested in the same manner. The emulsion in accordance with the invention possessed good sensitivity to X-ray intensifying screen radiation. The addition of the salts in accordance with the invention does not modify the sensitivity of the emulsion to X-ray radiation.

In accordance with the invention, I may use any of the tetraazaindene salts which are antifoggants for silver halide emulsions and which impart red sensitivity to the emulsion, for example, those described by Carroll et al. U.S. Patent 2,716,062 or Tinker et al. U.S. Patent 2,835,581, in the form of their alkali metal or ammonium salts. Particularly suitable are the 4-oxo or 4-hydroxy-tetraazaindenes, e.g., salts of the 4-hydroxy-1,3,3a,7-tetraazaindenes. These tetraazaindenes may contain various substituents, such as hydroxy, alkyl, amino and carboxyl. The salts may be conveniently prepared, for example, by reacting hydroxyl or carboxyl containing tetraazaindenes with an alkali metal hydroxide. The tetraazaindene salt may be employed in amounts of from 0.25 to 10, and preferably 1.0 to 5.0 g. per mole of silver.

Preferably, the noble metal salts which are employed are water soluble, although insoluble noble metal salts may be used. Representative salts of the noble metals, such as ruthenium, rhodium, palladium, iridium and platinum, which may be used include ammonium chloropalladate, potassium chloroplatinate and sodium chloropalladite. Advantageously, a soluble gold salt is used, potassium chloroaurate being particularly suitable. Other representative useful gold salts include potassium aurithiocyanate, auric trichloride and 2-aurosulfobenzothiazole methochloride. The noble metal salts are preferably employed in amounts of 1.0 to 5.0 mg. per mole of silver, although the most useful range is 0.25 to 10 mg. per mole of silver.

The independent addition to an emulsion of a noble metal salt subsequent to after-ripening of the emulsion lowers the sensitivity to red radiation. If desired, a noble metal salt may also be added to the emulsion before the after-ripening to increase sensitivity; advantageously, a gold salt is employed. In this instance, other sensitizers may be used with the gold (or noble metal) salts if desired, such as sulfur sensitizers, for example, those described in Sheppard et al. U.S. Patents 1,574,944, 1,623,499 and 2,410,689.

As indicated above, the tetraazaindene salt is added to the emulsion first and then the noble metal salt is incorporated therein. The salts must be added to the emulsion at the earliest, at the end of the after-ripening or second digestion, or anytime thereafter. It is necessary to add the tetraazaindene salt subsequent to the after-ripening step in the emulsion preparation since such salts would inhibit the effect of chemical sensitizers if added at an earlier stage of the emulsion preparation.

The addition of the tetrazaindene and noble metal salts is followed by a short period of digestion of the emulsion, such as from about 1-10 minutes at about 50° C. Advantageously, the salts are added during cooling of the emulsion after the second digestion, and while the emulsion is at about 50° C.

The invention is applicable to emulsions containing tetrazaindene salt antifoggants, which emulsions are not spectrally sensitized, or are spectrally sensitized only to the green region of the spectrum. The invention is particularly useful with medical X-ray emulsions which are not spectrally sensitized, but which may, of course, be chemically sensitized.

Emulsions in accordance with the invention have good fog stability and are substantially insensitive to the conventional red safelights employed in the photographic industry. Such safelights may be prepared, for example, by covering a 15 or 25 watt tungsten bulb with a filter which transmits light substantially only in the red region of the spectrum.

The invention has been described in detail with particular reference to preferred embodiments thereof, but it will be understood that variations and modifications can be effected within the spirit and scope of the invention as described hereinabove and as defined in the appended claims.

I claim:

1. In a method of preparing photographic silver halide X-ray emulsions containing tetrazaindene salt antifogant, which method comprises the steps of emulsification, removal of soluble salts and after-ripening, and separate additions following the after-ripening step of both a tetrazaindene salt and from 0.25 to 10 mg. per mole silver of a noble metal salt to said emulsion, the improvement wherein said additions following the after-ripening step are performed in the order of first adding said tetrazaindene salt and thereafter adding said noble metal salt

whereby red-safelight sensitivity of the emulsion is maintained below the red-safelight sensitivity that would obtain by opposite order of said additions.

2. An improved method defined by claim 1 further comprising a step of digesting the emulsion for a short time following the defined additions of tetrazaindene and noble metal salts.

3. A method defined by claim 1 wherein the defined tetrazaindene salt is a water-soluble 4-oxotetrazaindene salt and the defined noble metal salt is a water-soluble gold salt.

4. A method defined by claim 1 wherein the defined tetrazaindene salt is an alkali metal salt of a 4-hydroxy-1,3,3a,7-tetrazaindene and the defined noble metal salt is a water-soluble gold salt.

5. In a method of preparing photographic silver halide X-ray emulsions containing tetrazaindene salt antifogant, which method comprises the steps of emulsification, removal of soluble salts and after-ripening, the improvement which comprises first adding to the emulsion, while it is cooling subsequent to the after-ripening step, at about 50° C., about 1 g. per mole silver of 4-hydroxy-6-methyl-1,3,3a,7-tetrazaindene sodium salt, and following said first addition adding to the emulsion about 1.3 mg. per mole silver of potassium chloroaurate.

6. A photographic emulsion prepared in accordance with the method of claim 1.

#### References Cited

##### UNITED STATES PATENTS

|           |        |             |       |          |
|-----------|--------|-------------|-------|----------|
| 2,597,856 | 5/1967 | Damschroder | ----- | 96—108 X |
| 2,716,062 | 8/1955 | Carroll     | ----- | 96—109 X |

NORMAN G. TORCHIN, Primary Examiner.

R. E. FICHTER, Assistant Examiner.